

# United States Patent

[19]

[11] 3,909,426

Horodysky et al.

[45] Sept. 30, 1975

[54] EXTREME PRESSURE GREASE  
COMPOSITION

[75] Inventors: Andrew G. Horodysky; Henry  
Raich, both of Cherry Hill, N.J.

[73] Assignee: Mobil Oil Corporation, New York,  
N.Y.

[22] Filed: Oct. 3, 1973

[21] Appl. No.: 403,145

[52] U.S. Cl. .... 252/17; 252/41; 252/45  
[51] Int. Cl.<sup>2</sup> C10M 3/18; C10M 5/14; C10M 7/20;

C10M 7/24

[58] Field of Search ..... 252/17, 40, 41, 24, 45

## [56] References Cited

### UNITED STATES PATENTS

2,898,296 8/1959 Pattenden et al. .... 252/41

|           |         |                    |          |
|-----------|---------|--------------------|----------|
| 3,182,020 | 5/1965  | Davis .....        | 252/40.7 |
| 3,278,432 | 10/1966 | Davis .....        | 252/40.5 |
| 3,396,108 | 8/1968  | Caruso.....        | 252/18   |
| 3,574,111 | 4/1971  | Morway.....        | 252/17   |
| 3,681,242 | 8/1972  | Gilani et al. .... | 252/41   |
| 3,791,973 | 2/1974  | Gilani et al. .... | 252/41   |

Primary Examiner—Delbert E. Gantz

Assistant Examiner—I. Vaughn

Attorney, Agent, or Firm—Charles A. Huggett;  
Raymond W. Barclay; Benjamin I. Kaufman

[57]

## ABSTRACT

Grease compositions are provided comprising a lithium complex grease containing synergistic extreme pressure proportions of calcium acetate and dibenzyl disulfide.

1 Claim, No Drawings

## EXTREME PRESSURE GREASE COMPOSITION

## BACKGROUND OF THE INVENTION

## 1. Field of the Invention

This invention relates to grease compositions and, in one of its aspects, relates more particularly to grease compositions exhibiting improved extreme pressure properties. Still more particularly, in this aspect, the invention relates to grease compositions comprising lithium complex greases containing non-heavy metal additive mixtures as extreme pressure improvers.

## 2. Description of the Prior Art

Lithium complex greases have heretofore been widely employed in many industrial applications, and particularly in instances where a high-temperature grease is required as a lubricant. In order to achieve good extreme pressure properties, various additives have been incorporated in the grease, particularly materials containing heavy metal additives. Heavy metals, however, are known to function as oxidative promoters in lubricants. It has therefore become highly desirable to provide extreme pressure additives for these lithium complex greases which can impart good extreme pressure properties without the presence of heavy metal components, as heretofore employed. The term "lithium complex grease" is intended to denote greases having lithium salts of two or more carboxylic acids, e.g., a grease containing lithium salts of 12 hydroxystearic acid and a dibasic acid, such as azelaic, sebacic, adipic and similar acids as the complex thickening agent.

## SUMMARY OF THE INVENTION

It has now been found that marked improvement in extreme pressure properties can be imparted to lithium complex greases by incorporating into such greases, in an amount sufficient to achieve the desired extreme pressure properties, a mixture of calcium acetate and a sulfur-containing material. In this respect, it has been found that the aforementioned additive package for the lithium complex grease results in a marked improvement, from an oxidation standpoint, based upon the absence of undesirable heavy metals. In addition to exhibiting good extreme pressure characteristics, the novel greases are also found to be of highly desirable consistency, light color and the absence of objectionable odor.

Insofar as the sulfur-containing material is concerned, any sulfur-containing material may be employed in the additive combination, and particularly desirable are sulfur-containing materials selected from the group consisting of sulfur, alkyl sulfides, alkyl polysulfides, aromatic sulfides, aromatic polysulfides, sulfurized oils and fats. Where the sulfur-containing mate-

rial contains alkyl groups, each alkyl group preferably contains from 1 to 22 carbon atoms. Where the sulfur-containing material comprises a sulfide, these sulfides preferably contain from 1 to 10 sulfur atoms per mole.

5 Where the sulfur-containing material comprises sulfurized oils and sulfurized fats, these oils and fats preferably have a sulfur content of up to about 20%. Where the sulfur-containing material comprises a sulfurized oil, preferred sulfurized oils comprise mineral oils containing up to 5% sulfur. In a preferred modification, the sulfurized oils are selected from the group consisting of sulfurized lard oils and sulfurized sperm oils containing from 12 to 20% sulfur. In a still further preferred modification the sulfur-containing material comprises di-15 benzyl disulfide.

In its more specific aspects, the novel lithium complex greases of the present invention comprise calcium acetate in an amount from about 0.01% to about 50%, by weight, and from about 0.1% to about 30%, by 20 weight, of the sulfur-containing material. Particularly desirable grease compositions are represented by a lithium complex grease in which calcium acetate is present in an amount from about 0.2% to about 15%, by weight, and the sulfur-containing material, e.g. dibenzyl disulfide, is present in an amount from about 0.5% to about 15%, by weight. A more thorough description of the sulfur-containing materials employed in the novel grease compositions of the present invention is described in U.S. Pat. No. 3,278,432, issued Oct. 11, 1966. A wide variety of lubricating oils can be used as the vehicle for the novel greases of this invention, including both mineral and synthetic oils and particularly solvent-refined mineral oils.

## DESCRIPTION OF SPECIFIC EMBODIMENTS

The following examples and comparative data will serve to illustrate the novel greases of the present invention and to demonstrate their effectiveness as non-heavy metal lubricants possessing improved extreme pressure properties.

The standard test for determination of extreme pressure effects on grease compositions comprised the Timken Test O.K. Load, in pounds, according to ASTM D-2509.

In the comparative data and examples of the following table in which all components are expressed by weight, the base grease comprised a lithium complex grease viz., a lithium 12-hydroxystearic-azelaic acid grease (Example 1), in which were subsequently incorporated various additives and evaluated in accordance with the aforementioned Timken O.K. Load Test, as shown in the remaining examples. In each instance both the untreated and treated grease formulations exhibited light color and satisfactory odor.

55

TABLE

| Example | Grease Blend                                                              | Penetration<br>1/2 Scale | Timken Test<br>O.K. Load, Lbs.<br>ASTM D-2509 |
|---------|---------------------------------------------------------------------------|--------------------------|-----------------------------------------------|
| 1       | Lithium Complex<br>Base Grease                                            | 139/147                  |                                               |
| 2       | 2% Dibenzyl Disulfide<br>1.5% Chlorinated Paraffin<br>1.5% Sulfurized Fat | 148/151                  | < 40                                          |
| 3       | 2.5% Dibenzyl Disulfide<br>2.5% Chlorinated Paraffin                      | 140/                     | < 40                                          |
| 4       | 4% Dibenzyl Disulfide<br>4% Chlorinated Paraffin                          | 136/153                  | < 40                                          |

3  
TABLE -- Continued

| Example | Grease Blend                                                                                            | Penetration<br>1/8 Scale | Timken Test<br>O.K. Load, Lbs.<br>ASTM D-2509 |
|---------|---------------------------------------------------------------------------------------------------------|--------------------------|-----------------------------------------------|
| 5       | 4% Dibenzyl Disulfide<br>3% Chlorinated Paraffin<br>3% Sulfurized Fat                                   | 137/158                  | < 40                                          |
| 6       | 4% Dibenzyl Disulfide<br>3.5% Calcium Phenate                                                           | 157/170                  | < 40                                          |
| 7       | 4.5% Dibenzyl Disulfide<br>1% Chlorinated Paraffin<br>2% O,O-Dialkyl-S-Acyloxyalkyl Phosphoro-Dithioate | 152/155                  | < 40                                          |
| 8       | 8% Sulfurized Fat<br>2% Dibenzyl Disulfide                                                              | 158/172                  | < 40                                          |
| 9       | 10% Dibenzyl Disulfide                                                                                  | 136/155                  | < 40                                          |
| 10      | 10% Calcium Acetate<br>Dispersed in Mineral Oil                                                         | 146/158                  | < 40                                          |
| 11      | 5% Calcium Acetate<br>Dispersed in Mineral Oil<br>3% Dibenzyl Disulfide<br>2% Chlorinated Paraffin      | 146/158                  | > 50                                          |
| 12      | 5% Calcium Acetate<br>Dispersed in Mineral Oil<br>3% Chlorinated Paraffin                               | 144/156                  | < 40                                          |
| 13      | 5% Calcium Acetate<br>Dispersed in Mineral Oil<br>3% Dibenzyl Disulfide                                 | 147/155                  | > 60                                          |
| 14      | 3% Calcium Acetate<br>Dispersed in Mineral Oil<br>1.5% Dibenzyl Disulfide<br>1.5% Chlorinated Paraffin  | 144/153                  | 60                                            |
| 15      | 4% Calcium Acetate<br>Dispersed in Mineral Oil<br>2% Dibenzyl Disulfide<br>2% Chlorinated Paraffin      | 150/158                  | > 50                                          |
| 16      | 2% Dibenzyl Disulfide<br>1.5% Chlorinated Paraffin<br>1.5% Sulfurized Fat                               | 148/154                  | < 40                                          |

From the foregoing examples and comparative data, it will be apparent that the novel greases of the present invention exhibit markedly improved Timken O.K. Load properties. It should also be noted that other types of additives which provide further desirable properties may be added to the grease composition. These additives can include viscosity index improvers, pour point controlling agents, anti-oxidants and the like.

It will be understood that although the present invention has been described with preferred embodiments, various modifications and adaptations thereof may be

resorted to without departing from the spirit of the invention, as those skilled in the art will readily understand.

We claim:

1. A grease composition comprising a lubricating oil vehicle, a thickening amount of a lithium salt of 12-hydroxystearic acid and a lithium salt of an aliphatic dibasic acid, and synergistic extreme pressure proportions of calcium acetate and dibenzyl disulfide.

\* \* \* \* \*